

## UNITED STATES PATENT OFFICE

2,371,233

## RAYON

Wanda K. Farr, Yonkers, N. Y., assignor to The Chemical Foundation, Incorporated, a corporation of Delaware

No Drawing. Application June 6, 1939,  
Serial No. 277,625

3 Claims. (Cl. 260—217)

This invention relates to the production of an improved rayon.

The commercial production of cuprammonium silk, as is known, is based upon the original discoveries of John Mercer. Mercer, in common with his contemporaries, such as Schweizer, thought that cellulose was actually dissolved in cuprammonium solutions. For example, Mercer reported that cellulose fibers were "soluble" in a liquid obtained by dissolving hydrated cupric oxide to saturation in ammonia of sp. gr. 0.920 and diluting with three measures of water. On neutralizing with sulphuric acid, the organic matter was precipitated and later freed from copper by an excess of the acid. Schweizer similarly taught the art that with a sufficient excess of cuprammonium solution a true dissolution of cellulose occurred.

The commercial production of cuprammonium rayon did not begin until some thirty years after the original observation of the behavior of cotton fibers in cuprammonium hydroxide. This protracted delay was due to the technical difficulties in handling the spinning mixtures. Such mixtures were found to be unstable and tended to "separate." In the early efforts in this field even under the most favorable conditions, the regenerated fibers did not possess that degree of uniformity required by the trade.

Full scale commercial production of cuprammonium rayon was instituted only after the observation that "pretreatment" of the fibers overcame the earlier difficulties of separation. Such pretreatment consisted of a mercerization treatment usually by treatment with 18 per cent. sodium hydroxide at room temperature. It was found that such pretreated fibers dispersed uniformly in the cuprammonium hydroxide solution and the resulting spinning mixture, even in the high dilutions required for the finer fibers, remained stable and homogeneous throughout the entire spinning process. Following the original precepts of the art as to the "solubility" of cellulose in cuprammonium solution, this enhanced stability was attributed to an increased "solubility" of the mercerized fibers in the solvent. This concept of increased solubility has been substantially accepted down to the present time.

It has now been discovered that this concept is erroneous. It has definitely been established that, contrary to the generally accepted theory, true cellulose is not soluble in the typical cuprammonium solutions, and that enhanced stability of cuprammonium spinning mixtures is not due essentially to the modification of the cellulose. It

has been found, as a result of intensive, prolonged experimentation that the stability and spinability of cuprammonium vehicles containing cellulose is primarily a function of the characteristics of the non-cellulosic constituents of the fiber. In a word, it has definitely been determined that the spinning characteristics such as viscosity, stability, and the like, are largely determined by the colloidal characteristics of the non-cellulosic cementitious material natural with the true cellulose in cellulose membranes. In a more precise sense, it has been discovered that the stability of cuprammonium solutions is primarily a function of the speed of swelling or rate of imbibition of the non-cellulosic material of the fibrous starting material. It has been found that stability of cuprammonium spinning mixtures can be greatly enhanced, not by modification of the cellulose component but by positively inhibiting the swelling of the non-cellulosic component of the fibrous starting material.

The present invention, therefore, is based on the discovery that inhibition of such swelling markedly modifies the stability of the described spinning mixtures and specifically relates to improved methods of attaining or positively establishing such controlled inhibition, thereby insuring the concomitant or attendant advantages in commercial production of cuprammonium rayon.

30 The improved procedure which forms the basis of the present invention is based upon discoveries of the nature of the cellulose crystallite and its correlation with the amorphous cementitious material with which it is naturally associated in the cellulose membrane. To this extent the present application is a continuation in part of pending application of Wanda K. Farr, Serial No. 270,157, filed April 26, 1939.

As is fully described in the application referred to, it has been discovered that the cellulose component of the cell membrane of the cotton fiber, which is in the form of individually distinct, ellipsoid particles, does not dissolve in a standard solution of cuprammonium hydroxide, as has been popularly supposed. In experiments recorded in the cross-referenced application, cellulose membranes of different types were dispersed in standard cuprammonium solutions. By special technique, involving among others, the use of such factors as critical illumination, the slit ultra microscope and extremely small cross sections of specimens, it definitely was established that the action in such solutions involved essentially the extenuation of the cementitious non-cellulosic material and the concomitant disintegration

of the cellulose from its original condition of a closely packed, definitely oriented fibrous structure into a random colloidal dispersion of the ultimate cellulose particles (1.5 x 1.1 mu). As recorded in that application, the true cellulose may be separated from the colloidal continuous phase and such separated cellulose re-dispersed (free from the associated cementitious material) in standard cuprammonium solutions. Similarly, by improved methods, as described in said co-pending application, the cementitious material may be separated and recovered from the cellulose.

It was found that the true cellulose itself had little if any effect upon the viscosity of cuprammonium solutions; that such cellulose was a precise or definite entity and that, however the cellulose was produced, it had substantially no effect upon the viscosity of cuprammonium hydroxide. It was found conversely, and most unexpectedly in view of the teachings of the art, that the determinant in establishing the increased viscosity of cuprammonium solutions was not the quantity of the cellulose in the solution but was the cementitious material, and that the viscosity of a cuprammonium system was a direct function of the quantity of this cementitious material contained in the solution. As a result of microscopic examination as well as chemical analysis, as for example by uronic anhydride determinations, it was determined that the characteristics of this cementitious material placed it in the category of what is generally known as "pectic" substance.

The results described in the application referred to fundamentally alter the previous conception of the behavior of both untreated and purified cell membranes in solutions of cuprammonium hydroxide. It is obvious from the earlier literature that this viscosity-producing characteristic of the pectous material has been entirely overlooked, as well as the fact that the cellulose, per se, exists in a cuprammonium solution, not as a dissolved substance but as a dispersed colloidal phase.

Upon these findings the present invention is based. Under the present invention the stability of cuprammonium spinning solutions may be enhanced and definitely established by suitably modifying the component which engenders instability, namely, the non-cellulosic pectous component. In brief, the present invention relates to a method of increasing the stability of cuprammonium spinning solutions not by any attempt at modification of cellulose itself but by inhibiting the swelling action of the intercrystalline, cementing material.

In experimentations in this field, it was observed that when very thin cross sections (2 to 3 mu) of cotton fibers were treated with cuprammonium hydroxide, some striking effects were produced. If these sections were previously untreated the plastic and viscous cementing material, existing as an intercrystalline, and apparently continuous phase, swelled most rapidly and almost explosively. Such swelling could, however, be readily inhibited by pretreating the sample with a slight amount of strong sodium hydroxide, or, preferably, potassium hydroxide. Such a pretreated example swelled very gradually and three stages of the action were readily discernible: first, an early stage in which there was a general increase in the diameter of the cross section of the specimen due to the imbibition or expansion of the cementing substance; a later stage in which the lamellae making up the fiber separated from each

other to the extent that they were readily discernible; and a final stage in which the lamellae themselves disintegrated into cellulose particles of colloidal dimensions which are randomly dispersed in the swollen colloid matrix. These cellulose particles, which had the approximate dimensions 1.5 x 1.1 mu, exhibit the Tindall effect, Browning movement, and other characteristics of colloidal dispersions; and as a result of these findings it was determined that the stability of a spinning mixture of cuprammonium hydroxide is due, not to increased solubility of the cellulose, or in fact any solubility of the cellulose whatever, but to one of increased colloidal stability of the cementing material. It was definitely established, for example, that the cellulose particles, as such, are present as a dispersed phase in the cuprammonium solution whether they had been previously mercerized or not. Under the present invention, this discovery is utilized to improve cuprammonium spinning solutions by the simple expedient of pretreating the fibers, not with a reagent which insures mercerization or necessarily under mercerizing conditions but with a reagent and under conditions which are chosen so as selectively to inhibit the swelling function of the pectic substance.

In one preferred modification it has been found that such inhibition may be secured with cheap reagents, e. g. sodium hydroxide or potassium anhydride in relatively low concentrations and at relatively low temperatures as distinguished from the relatively elevated temperatures which had been thought necessary in the past in order to secure mercerization.

In a typical case, the desired inhibition of the rapid swelling of the cementitious material and the attainment of the concomitant desirable stability of the colloidal cementing phase, may readily be secured by treating the cellulosic starting material, e. g. cotton fibers, with a sodium hydroxide solution, the activity of which is controlled to secure a specific or definite effect on the cementitious phase without any effort to obtain mercerization of the fibers. For example, the fibrous starting material may be treated with sodium hydroxide solutions of from 18% down to 10% and lower, which solutions are preferably maintained at a low temperature, i. e., of the order of 4° C. It will be observed that this type of treatment is essentially different from the prior art methods in which sodium hydroxide solutions of 18% or higher were employed at elevated temperatures so as chemically to modify the cellulose. Under the conditions of the present invention, while sodium hydroxide may be employed, it is used under conditions controlled preferentially to modify a physicochemical characteristic of a non-cellulosic component of the starting material and not as in the prior art, to chemically change the cellulose.

Since the fibrous or cellulosic starting materials which are used in the production of cuprammonium silk may vary considerably, the conditions of the swelling inhibition treatment may be modified to secure the desired degree of colloidal stability for the particular material used. The relationship of concentration of the reagent and the time and temperature of the treatment may thus be definitely correlated with the particular starting material.

After the desired degree of pretreatment, the fibrous material may be freed of the alkali hydroxide, washed, and then dispersed in a typical cuprammonium solution. The resulting disper-

sion may then be ejected into water, stretched, and then treated in the acid coagulating bath in the usual manner.

It will be understood that within the broad concept of the invention, a number of specifically different materials or reagents may be employed to effect the desired modification of the external or cementitious phase. Any material which functions to operate on the non-cellulosic material to reduce its swelling tendency and to colloidally stabilize it, is suitable.

In experimentation in this field it has been found that a particularly efficacious method of producing improved cellulose dispersions, as for example a dispersion of cellulose in cuprammonium hydroxide, comprises a treatment with a relatively weak solution of nitric acid followed by treatment with a caustic soda solution. In a preferred mode of operation, for the production of cuprammonium rayon, the cellulosic starting material is treated with a solution of 1% nitric acid at about room temperature for a period of from approximately 10 to 20 hours. During the period the cellulosic material may be agitated continuously or intermittently. After this period of contact the nitric acid solution is drained, the cellulose washed with water and then treated with a caustic soda solution of approximately 10% concentration at a temperature from room temperature down to about 4° C. Thereafter the cellulose may be dispersed in a cuprammonium hydroxide solution in the usual manner.

The treatment with nitric acid appears to have a critical or specific beneficial effect. The outer limiting membrane of cellulose fibers, as is known, is of a different chemical constituency from the remainder. This outer membrane contains a protective substance, generally designated as cutin. The material is insoluble in the reagents generally employed in the pretreatment and dispersion of cellulose and in many instances appears in the final product, that is to say, the extruded rayon filament or sheet. Such material occurs in the filament as a dispersed impurity and causes considerable difficulty in dyeing in that it does not respond or react to the dye as does the regenerated cellulose thus giving an imperfect product. The nitric acid treatment appears to selectively extract this constituent or fraction from the cellulosic material while at the same time beneficially modifying the colloidal characteristics of the intercrystalline or pectous phase insuring greater colloidal stability.

It has been ascertained that the described pretreatment with weak nitric acid is of wide utility in the rayon field. As noted above the described chemical constituent which occurs in the outer limiting membrane of cellulose fibers is quite refractory. As a result of numerous tests, it has been discovered that in many circumstances this constituent appears in certain viscose rayon fibers. In other words this particular substance is resistant even to the action of the 18% caustic solution used in preparing the alkali cellulose for

xanthation. Under one phase of the present invention viscose rayons may considerably be improved, especially in respect to uniform dyeing, by selectively extracting this characterizing constituent of the outer limiting membrane of the cellulose fiber prior to dispersion of the cellulose. A simple and effective method of accomplishing this is to subject the cellulosic material to the described extraction with nitric acid. Preferably this is done prior to the formation of the alkali cellulose. The extraction with the nitric acid solution may be effected by a simple batch immersion treatment or by continuously recirculating the weak nitric acid solution through a mass of the cellulosic material. When such a treatment is employed it is found that the undesirable constituents are removed from the cellulose. Viscose rayons produced from such pretreated cellulose are characterized by an improved uniformity with respect to dyeing.

It will be appreciated that the term "cutin" herein applied to the undesired constituent of the cellulose membrane is used in a generally descriptive rather than a strictly scientific sense. This material probably is not a single chemical individual but may be a mixture of compounds. Researches to date indicate that it is comprised largely of suberin. With respect to the present disclosure, the term cutin is intended to comprehend those constituents such as the water resistant wax-like components which characteristically distinguish the outer limiting membrane from the remainder of the fiber.

Hence while preferred pretreating agents have been described, it is to be understood that these are chosen to illustrate an effective though not the exclusive method of procedure. The invention resides not so much in the use of particular reagents at definite concentrations and temperature, but primarily in the discovery of the essential role of the non-cellulosic phase and for the practical methods of modifying its colloidal characteristics so as to insure the proven new results.

Having thus described my invention, I claim:

45 1. In the production of viscose rayons that improvement which comprises extracting cotton cellulose, prior to alkalization at room temperature, with a solution of nitric acid of approximately 1% strength for a time sufficient to selectively extract the cutin-like component of the material.

50 2. In the production of viscose rayons that improvement which comprises extracting cotton cellulose at substantially room temperature with a 1% solution of nitric acid for a period of the order of 15 hours to extract cutin-like substances without substantial decomposition of the other components of the starting material.

55 3. In the production of viscose rayons that improvement which comprises extracting cotton fibers with a 1% solution of nitric acid at room temperature for a period of from approximately 10 to 20 hours.

WANDA K. FARR.